

Patented May 4, 1948

2,440,969

38

## UNITED STATES PATENT OFFICE

2,440,969

## PROTECTIVELY COATED FERROUS METAL SURFACES AND METHOD OF PRODUCING SAME

Victor Charles John Nightingall, deceased, late of Heidelberg, Victoria, Australia, by Ruth Valencia Nightingall, Aubrey Mitchell Old, and Charles Montefiore Gladstone Nightingall, executors, Melbourne, Victoria, Australia, assignors to Di-Met Proprietary Limited, West Melbourne, Victoria, Australia, a company of Victoria, Australia

No Drawing. Application January 7, 1948,  
Serial No. 1,072

10 Claims. (Cl. 117—127)

**1** This invention relates to protective coatings for metal surfaces and, more particularly, to hard protective coatings for the surfaces of ferrous metal articles. The invention contemplates a novel method of producing such coatings on a ferrous metal surface and the resulting article having on its surface such a hard protective coating.

Protective coatings for metal surfaces must meet several requirements if they are to be considered effective. Such coatings must be continuous and impervious to corrosive elements, must be sufficiently hard to withstand the normal abrasion and mechanical shock to which metal articles are frequently subjected, and must have a high degree of adherence to the surface of the metal article. If a coating does not adequately meet these requirements, it fails to qualify as a protective coating. This is particularly true with respect to protective coatings for ferrous metal articles where a single flaw in the coating will permit widespread corrosion and even disintegration of the ferrous article beneath the coating.

The method of the present invention contemplates the provision of a hard protective coating on a ferrous metal surface in such manner that the coating meets each of the aforementioned requirements. The method of producing such a coating on a ferrous metal surface in accordance with the invention comprises applying to the surface a coating of a composition comprising finely divided metallic zinc and finely divided lead oxide incorporated in an aqueous solution containing an alkali silicate and sodium bicarbonate, and preferably also boracic acid, and drying the applied coating. The coating obtained by this method is extremely hard, protective, abrasion-resistant, adherent and water insoluble. It is particularly effective as a protective corrosion-resistant coating on the surface of ferrous metals such as iron and steel.

The amount of finely divided zinc used in the coating composition may range from about 100% to 350% by weight of the alkali silicate solution and is preferably such as to comprise between about 140% to 280% by weight of the solution. A particularly effective composition comprises about 200% by weight of the silicate solution. The finely divided zinc may advantageously comprise fine zinc dust of pigment particle size as free of zinc oxide as possible.

**2** The quantity of finely-divided lead oxide used in making up the composition of the invention may range from about 5% to 20% by weight of the zinc used. The lead oxide promotes drying or insolubilization of the coating composition, and makes possible complete drying and insolubilization of the coating by simple air-drying. The lead oxide further appears to increase the hardness and abrasion resistance of the dry coating. About 5% lead oxide by weight of the zinc used appears to be the smallest effective amount of lead oxide. An excess of lead oxide above about 20% by weight of the zinc unduly dilutes the zinc and tends to impair the corrosion-resistant effectiveness of the coating. Particularly effective results have been obtained using amounts of lead oxide ranging from about 10% to 20% by weight of the zinc. Although the lead oxide is preferably added in the form of red lead ( $Pb_3O_4$ ) because of its commercial availability and favorable cost, litharge ( $PbO$ ) and lead suboxide ( $Pb_2O$ ) have been used successfully within the above-mentioned ranges.

The alkali silicate solution may be made up of sodium silicate, potassium silicate, lithium silicate, or a mixture of such silicates, in the form of an aqueous solution having a specific gravity of approximately 1.3 (i. e., around 30% by weight of alkali silicate). Effective coating compositions may be made up with alkali silicate solutions of both higher and lower specific gravities, and satisfactory results have been obtained in practice with solutions containing from about 20% to 40% by weight of the alkali silicate. The sodium silicate, for example, may be of any of the commonly marketed ratios of  $Na_2O$  to  $SiO_2$ , which generally range from 1:1.7 to 1:3.9, but particularly satisfactory drying characteristics are obtained with a  $Na_2O$  to  $SiO_2$  ratio between about 1:2.4 and 1:2.6.

To the solution of alkali silicate is added sodium bicarbonate in amount ranging from about 0.1% to about 0.8% by weight based on the weight of the alkali silicate solution. The actual amount of sodium bicarbonate required in the silicate solution to effect the formation of an insoluble complex silicate in accordance with the invention varies with the amount of free alkali in the silicate solution which must be neutralized by the bicarbonate before the unconsumed bicarbon-

ate is available to produce the desired complex silicate. The amount of free alkali to be neutralized depends to some extent upon the ratio of  $\text{Na}_2\text{O}$  to  $\text{SiO}_2$  in the silicate and upon the concentration of the silicate solution. The amount of free alkali to be neutralized also appears to vary with the amount of zinc present in the composition, and, of course, depends upon whether boracic acid is used in preparing the coating composition as hereinafter more fully discussed. Approximately 0.1% sodium bicarbonate appears to be the smallest effective amount which can be used in accordance with the invention, and this lower limit can be obtained only by the use of the maximum permissible amount of boracic acid. Amounts of sodium bicarbonate substantially in excess of 0.8% by weight of the silicate solution can be tolerated, either in the presence or absence of boracic acid, without precluding the formation of an insoluble coating when the applied composition is dried. However, such excessive amounts of sodium bicarbonate are detrimental to the appearance of the coating because they promote the formation of a bloom on its surface and are detrimental to the effectiveness of the coating because they tend to impart porosity thereto.

The sodium bicarbonate may be added to the silicate solution in the solid form or in the form of an aqueous solution. The latter form is preferred because it facilitates complete dissolution and uniform dispersion of the sodium bicarbonate in the alkali silicate solution. The bicarbonate solution is advantageously one which is saturated with the bicarbonate at the temperature of the silicate solution to which it is added (generally room temperature). For example, the addition of about 12 parts by volume of a sodium bicarbonate solution saturated at 60° F. to 100 volumes of an alkali silicate solution having a specific gravity of about 1.3 is equivalent to the addition of about 0.8% of sodium bicarbonate by weight of the silicate solution. Smaller quantities of the bicarbonate solution may be added to the silicate solution when less free alkali is present to be neutralized by the bicarbonate as explained hereinabove.

Boracic acid is preferably also added to the alkali silicate solution in an amount sufficient to react with the bulk of the free alkali in the solution but insufficient to cause precipitation of silicic acid. To the extent that the free alkali is neutralized by the boracic acid, the required amount of sodium bicarbonate may be reduced in accordance with the principle heretofore explained. For example, when about 0.2% by weight of boracic acid based on the weight of the solution is added to a sodium silicate solution having a specific gravity of about 1.3 and a  $\text{Na}_2\text{O}$  to  $\text{SiO}_2$  ratio of about 1:2.4, the amount of sodium bicarbonate required in accordance with the invention may be reduced to about 0.2% by weight of the silicate solution. Larger or smaller amounts of boracic acid may be used with advantage, the only limitation being that it be not added in amount sufficient to cause precipitation of silicic acid from the silicate solution. The boracic acid may be added in the solid form, although it is preferred to add the boracic acid in the form of a substantially saturated aqueous solution in order to facilitate dissolution thereof in the silicate solution. In addition to its effect in reducing the amount of sodium bicarbonate required, the inclusion of boracic acid in the coat-

ing composition effects a substantial increase in the hardness of the dry coating.

In forming a hard protective coating on a metal surface in accordance with the invention, the metal surface such as iron or steel is preferably first cleaned to remove all scale, rust, dirt, and the like. The metal surface may be cleaned in a pickling bath such as a solution of phosphoric acid or sulphuric acid, followed by appropriate rinsing. The surface may also be cleaned by sand blasting, buffing, or other mechanical means. The surface of the metal is then coated with the composition comprising the finely divided zinc and lead oxide incorporated in the aforesaid aqueous silicate solution. The composition may be applied to the metal surface either by dipping, brushing, spraying, or the like. The dipping procedure produces a relatively heavy coating which varies in thickness with the viscosity of the coating composition. The brushing and spraying procedures are more readily controlled and can be used to provide any coating thickness ranging from very thin coatings to heavy coatings of excellent physical characteristics.

The composition applied to the metal surface is then dried under conditions such as to substantially dehydrate the coating composition. This result may be accomplished by permitting the applied composition to dry for a period of at least twenty-four hours, and preferably for a period of about 36 to 48 hours, in an atmosphere of normal temperature and humidity. Excessive moisture in the atmosphere, as evidenced by high humidity, or rain or dew, impedes the drying step and interferes with the production of a hard, protective coating. The drying may be expedited with particularly effective results by heating the applied coating to a temperature of about 180 to 500° F. for a period of about 2 to 12 hours, the heating period depending upon the heating temperature used.

The chemical reactions which take place within the applied coating composition during the drying stage are obscure, although there is evidence that a mixture of silicates or complex silicates, or both, are formed. It appears that the lead oxide has a catalytic action which is particularly important when dehydration is effected at normal temperatures. Additionally, however, the lead oxide improves the properties of the coatings obtained either by air-drying or by heating to a temperature of 180° F. or higher. It is believed that carbon dioxide released from the bicarbonate reacts to produce carbonate of zinc or other zinc compounds which in turn react with the sodium silicate or silicic acid precipitated by the carbon dioxide to form a complicated zinc silicate. These suggested reactions, however, represent only the first stage of the formation of the ultimate coating, as further advantageous but obscure changes occur slowly over a period of one or two years or more.

The boracic acid incorporated in the solution reduces the alkalinity thereof and thus the carbon dioxide subsequently released from the bicarbonate is more fully available to react with the zinc, since only a minor portion of the bicarbonate is then required for completely neutralizing the alkalinity of the silicate solution. The boracic acid presumably reacts with the free alkali to form borax which latter, it is thought, has a useful fluxing effect.

The tenacity with which the dried coating adheres to the metal surface to which it has been

2,440,969

5

applied suggests that some reaction with the ferrous metal surface takes place, such as the formation of an iron silicate. Whatever reactions actually take place, the applied composition forms a protective, hard, abrasion-resistant, adherent coating by the end of the drying period, that is, by the time the applied composition is substantially dehydrated. It must be understood, however, that the dehydration referred to herein comprises the removal of free moisture from the applied composition and not necessarily the complete removal of water chemically combined with the other ingredients of the coating composition.

The following specific examples will serve to further illustrate the practice of the invention:

I

An aqueous solution of sodium silicate and sodium bicarbonate was prepared by dissolving in water a sufficient quantity of sodium silicate having a  $\text{Na}_2\text{O}$  to  $\text{SiO}_2$  ratio of about 1:2.4 to form a solution having a specific gravity of approximately 1.3, and by then adding thereto a saturated solution of sodium bicarbonate (i. e., saturated at 60° F.) in the proportion of 12 parts by volume of the sodium bicarbonate solution to 100 parts by volume of the silicate solution. This addition corresponds to about 0.8% sodium bicarbonate by weight of the silicate solution. Sufficient boracic acid was then incorporated in the solution to substantially completely remove free alkali therefrom while avoiding precipitation of silicic acid. About 5½ pints (Imperial) of this solution weighing about 9 pounds were placed in a mechanical mixing machine and about 20 pounds of very fine zinc dust substantially free of zinc oxide were added. The mixture was then worked in the mixing machine for about 4 minutes, after which approximately 10% of red lead by weight of the solution (i. e., about 1 pound) was added, and mixing was continued for an additional 4 to 10 minutes. The composition was promptly applied to a metal surface with a brush and the applied coating was allowed to dry in the air at temperate humidity and temperature conditions for a period of about 36 hours. The resulting coating was hard, insoluble, adherent, and abrasion-resistant and fully protected the metal surface against corrosion by outdoor atmospheric conditions.

II

An aqueous solution of sodium silicate was prepared having a specific gravity of approximately 1.3 and a  $\text{Na}_2\text{O}$  to  $\text{SiO}_2$  ratio of 1:2.4. To 100 gallons (Imperial) of this solution were added 2.5 pounds of boracic acid, and 2.5 pounds of sodium bicarbonate, both in the form of saturated solutions at room temperature. About 6 pints (Imperial) of the resulting solution, weighing approximately 10 pounds, were placed in a mechanical mixer and 20 pounds of commercial zinc dust were added. After a few minutes interval 2 pounds of red lead were added and mixing was continued for an additional period of several minutes. The coating obtained by air-drying the composition applied to a steel surface was hard, insoluble, adherent and abrasion-resistant and fully protected the steel surface against corrosion.

III

An aqueous solution of sodium silicate having a  $\text{Na}_2\text{O}$  to  $\text{SiO}_2$  ratio of 1:2.4 was prepared having a specific gravity of about 1.3. About 10.5

6

pounds of sodium bicarbonate were added to 1300 pounds of the silicate solution by adding 12 gallons (Imperial) of a solution of sodium bicarbonate saturated at 60° F. to 100 gallons (Imperial) of the sodium silicate solution. About 20 pounds of zinc dust and 2 pounds of red lead were incorporated in 6 pints (Imperial) of the silicate-bicarbonate solution and the resulting composition was applied with a brush to a steel surface. The coating was allowed to dry in the open atmosphere and formed a hard, insoluble, abrasion-resistant and corrosion-resistant coating on the steel surface.

The aqueous solution of alkali silicate containing either sodium bicarbonate alone or sodium bicarbonate and boracic acid is stable over a long period of time. Upon the addition of the metallic zinc and lead oxide to the silicate solution, however, the mixture becomes unstable in that it tends to set. The time required for this setting to become objectionable ranges from about 10 minutes in an atmosphere at a temperature substantially in excess of 90° F. to about 10 hours in a cold atmosphere. Accordingly, the solid ingredients of the composition (the finely divided zinc and the lead oxide) should not be incorporated in the silicate solution until just before the composition is to be applied to the metal surface to be protected. In general, the coating composition of the invention should be applied to the ferrous metal surface within about 15 to 45 minutes after incorporation of the metallic zinc and lead oxide in the silicate solution. For this reason, it is expedient to prepare the silicate solution in large quantities but to add the solid ingredients to only so much of the silicate solution as will make up a volume of coating composition which can be applied to the ferrous surface within the aforementioned time limit. The zinc and lead oxide may be added separately to the silicate solution or they may be combined in the desired proportion for incorporation in the silicate solution as a single addition. Thus, the coating composition is advantageously packaged for field and other use in the form of two complementary units (one the liquid vehicle and the other the solid ingredients) adapted, when their contents are admixed, to produce the composition of the invention in condition for immediate use.

It will be understood also that, if desired, pigments and/or fillers may be included in the above mentioned coating mixtures either to provide increased body or to modify the appearance, whether as to color or otherwise, of the resultant coatings.

This application is a continuation-in-part of an application for Letters Patent of the United States, filed March 18, 1947, Serial No. 735,534, now abandoned, which application was a continuation-in-part of an application for Letters Patent of the United States, filed July 3, 1945, Serial No. 603,116, both of said applications having been filed by Victor Charles John Nightingall.

65 It is claimed:

1. The method of producing a hard protective coating on a ferrous metal surface which comprises applying to the surface a coating of a composition comprising finely divided metallic zinc and finely divided lead oxide incorporated in an aqueous solution of an alkali silicate and sodium bicarbonate, the aqueous solution containing about 20% to 40% by weight of the alkali silicate and about 0.1% to 0.8% by weight of sodium bicarbonate, the zinc being present in

amount of about 100% to 350% by weight of said solution and the lead oxide being present in amount of about 5% to 20% by weight of the zinc, and drying the applied coating.

2. The method of producing a hard protective coating on a ferrous metal surface which comprises applying to the surface a coating of a composition comprising finely divided metallic zinc and finely divided lead oxide incorporated in an aqueous solution of an alkali silicate and sodium bicarbonate, the aqueous solution containing about 30% by weight of the alkali silicate and about 0.2% to 0.8% by weight of sodium bicarbonate, the zinc being present in amount of about 140% to 280% by weight of said solution and the lead oxide being present in amount of about 10% to 20% by weight of the zinc, and drying the applied coating.

3. The method of producing a hard protective coating on a ferrous metal surface which comprises applying to the surface a coating of a composition comprising finely divided metallic zinc and finely divided lead oxide incorporated in an aqueous solution of an alkali silicate and sodium bicarbonate, the aqueous solution containing about 30% by weight of the alkali silicate and about 0.8% by weight of sodium bicarbonate, the zinc being present in amount of about 200% by weight of said solution and the lead oxide being present in amount of about 10% by weight of the zinc, and drying the applied coating.

4. The method of producing a hard protective coating on a ferrous metal surface which comprises applying to the surface a coating of a composition comprising finely divided metallic zinc and finely divided lead oxide incorporated in an aqueous solution of an alkali silicate containing sodium bicarbonate and boracic acid, the aqueous solution containing about 20% to 40% by weight of the alkali silicate, about 0.1% to 0.8% by weight of sodium bicarbonate, and the boracic acid being added to the solution in amount sufficient to react with the bulk of the free alkali in the solution but insufficient to cause precipitation of silicic acid, the zinc being present in amount of about 100% to 350% by weight of said solution and the lead oxide being present in amount of about 5% to 20% by weight of the zinc, and drying the applied coating.

5. The method of producing a hard protective coating on a ferrous metal surface which comprises applying to the surface a coating of a composition comprising finely divided metallic zinc and finely divided lead oxide incorporated in an aqueous solution of an alkali silicate containing sodium bicarbonate and boracic acid, the aqueous solution containing about 30% by weight of the alkali silicate, about 0.2% to 0.8% by weight of sodium bicarbonate, and the boracic acid being added to the solution in amount sufficient to react with the bulk of the free alkali in the solution but insufficient to cause precipitation of silicic acid, the zinc being present in amount of about 140% to 280% by weight of said solution and the lead oxide being present in amount of about 10% to 20% by weight of the zinc, and drying the applied coating.

6. The method of producing a hard protective coating on a ferrous metal surface which comprises applying to the surface a coating of a composition comprising finely divided metallic zinc and finely divided lead oxide incorporated in an aqueous solution of an alkali silicate con-

taining sodium bicarbonate and boracic acid, the aqueous solution containing about 30% by weight of the alkali silicate, about 0.2% by weight of sodium bicarbonate, and about 0.2% by weight of boracic acid, the zinc being present in amount of about 200% by weight of said solution and the lead oxide being present in amount of about 10% by weight of the zinc, and drying the applied coating.

10 7. A ferrous metal article having on the surface thereof a hard protective coating resulting from the application thereto and the drying thereon of a composition comprising finely divided metallic zinc and finely divided lead oxide incorporated in an aqueous solution of an alkali silicate and sodium bicarbonate, the aqueous solution containing from about 20% to 40% by weight of the alkali silicate and from about 0.1% to 0.8% by weight of the sodium bicarbonate, the zinc being present in amount of about 100% to 350% by weight of said solution, and the lead oxide being present in amount of about 5% to 20% by weight of the zinc.

25 8. A ferrous metal article having on the surface thereof a hard protective coating resulting from the application thereto and the drying thereon of a composition comprising finely divided metallic zinc and finely divided lead oxide incorporated in an aqueous solution of an alkali silicate and sodium bicarbonate, the aqueous solution containing about 30% by weight of the alkali silicate and about 0.8% by weight of the sodium bicarbonate, the zinc being present in amount of about 200% by weight of said solution, and the lead oxide being present in amount of about 10% by weight of the zinc.

30 9. A ferrous metal article having on the surface thereof a hard protective coating resulting from the application thereto and the drying thereon of a composition comprising finely divided metallic zinc and finely divided lead oxide incorporated in an aqueous solution of an alkali silicate, sodium bicarbonate and boracic acid, the aqueous solution containing from about 20% to 45 40% by weight of the alkali silicate, from about 0.1% to 0.8% by weight of the sodium bicarbonate, and an amount of boracic acid sufficient to react with the bulk of the free alkali in the solution but insufficient to cause precipitation of silicic acid, the zinc being present in amount of about 100% to 350% by weight of said solution, and the lead oxide being present in amount of about 5% to 20% by weight of the zinc.

50 10. A ferrous metal article having on the surface thereof a hard protective coating resulting from the application thereto and the drying thereon of a composition comprising finely divided metallic zinc and finely divided lead oxide incorporated in an aqueous solution of an alkali silicate, sodium bicarbonate and boracic acid, the aqueous solution containing about 30% by weight of the alkali silicate, about 0.2% by weight of the sodium bicarbonate, and about 0.2% by weight of boracic acid, the zinc being present in amount of about 200% by weight of said solution, and the lead oxide being present in amount of about 10% by weight of the zinc.

RUTH VALENCIA NIGHTINGALL,  
AUBREY MITCHELL OLD,  
CHARLES MONTEFIORE GLADSTONE  
NIGHTINGALL,  
Executors of the Estate of Victor Charles John  
Nightingall, Deceased.